

# United States Patent [19]

Oxman et al.

[11] Patent Number: 4,735,632

[45] Date of Patent: Apr. 5, 1988

[54] COATED ABRASIVE BINDER CONTAINING  
TERNARY PHOTINITIATOR SYSTEM

[75] Inventors: Joel D. Oxman, Minneapolis; F.  
Andrew Ubel, III, St. Paul; Eric G.  
Larson, White Bear Lake, all of  
Minn.

[73] Assignee: Minnesota Mining and  
Manufacturing Company, St. Paul,  
Minn.

[21] Appl. No.: 34,066

[22] Filed: Apr. 2, 1987

[51] Int. Cl.<sup>4</sup> ..... B24D 11/00

[52] U.S. Cl. ..... 51/295; 51/293;  
51/298; 430/332

[58] Field of Search ..... 51/293, 295, 298;  
430/332, 340

## [56] References Cited

### U.S. PATENT DOCUMENTS

|           |         |              |         |
|-----------|---------|--------------|---------|
| 3,729,313 | 4/1973  | Smith        | 430/332 |
| 4,011,063 | 3/1977  | Johnston     | 51/295  |
| 4,047,903 | 9/1977  | Hesse et al. | 51/295  |
| 4,126,428 | 11/1978 | Rude         | 51/295  |

|           |         |                  |        |
|-----------|---------|------------------|--------|
| 4,240,807 | 12/1980 | Kronzer          | 51/295 |
| 4,298,356 | 11/1981 | Teschner et al.  | 51/295 |
| 4,457,766 | 7/1984  | Caul             | 51/298 |
| 4,547,204 | 10/1985 | Caul             | 51/298 |
| 4,642,126 | 2/1987  | Zador et al.     | 51/298 |
| 4,652,274 | 3/1987  | Boettcher et al. | 51/293 |

Primary Examiner—Paul Lieberman

Assistant Examiner—Willie J. Thompson

Attorney, Agent, or Firm—Donald M. Sell; James A.  
Smith; David R. Cleveland

[57]

## ABSTRACT

Coated abrasive binders made from a photocurable addition-polymerizable composition containing a free-radically-polymerizable monomer and a photoinitiator system containing (i) an arylidonium salt, (ii) a sensitizing compound, and (iii) an electron donor having an oxidation potential that is greater than zero and less than or equal to that of p-dimethoxybenzene (1.32 volts vs. S.C.E.). The binders cure rapidly and deeply under ultraviolet or visible light, even when filled with large amounts of mineral grain or with coarse grades of minerals.

24 Claims, No Drawings

COATED ABRASIVE BINDER CONTAINING  
TERNARY PHOTONITIATOR SYSTEM

## TECHNICAL FIELD

This invention relates to coated abrasives made using photochemically initiated binders.

## BACKGROUND ART

When coated abrasives are made from conventional binders such as hide glue, varnish or phenolic resins, the manufacturing process can be both energy-intensive and time-consuming. For example, the widely-used phenolic binders must be dried at high temperatures for long times (e.g., at least about 2 hours at 90° C. (195° F.) for cure of phenolic size coatings). In an effort to reduce energy consumption and increase throughput, coated abrasive manufacturers have investigated electron-beam ("E-beam")-curable binders and photochemically-curable binders, e.g., as described in recently-issued U.S. Pat. Nos. 4,642,126 and 4,652,274.

A general shortcoming of radiation curing as applied to coated abrasive manufacture lies in the inherent difficulty of curing behind an abrasive grain in highly-filled or thick-section coated abrasive products. As a result, the abrasive grains may be poorly adhered on the backing, with concomitant poor product performance. Combinations of E-beam cure and thermally-initiated cure have been employed to overcome this shortcoming; however, such an approach still represents a compromise solution that can require considerable time and energy for completion of a thermal cure cycle.

Aryliodonium salts have been previously described for use as photoinitiators in addition-polymerizable compositions. References relating to such compositions include U.S. Pat. Nos. 3,729,313, 3,741,769, 3,808,006, 4,228,232, 4,250,053 and 4,428,807; H. J. Timpe and H. Baumann, *Wiss. Z. Tech. Hochsch. Leuna-Merseburg*, 26, 439 (1984); H. Baumann, B. Strehmel, H. J. Timpe and U. Lammel, *J. Prakt. Chem.*, 326 (3), 415 (1984); and H. Baumann, U. Oertel and H. J. Timpe, *Euro Polym. J.*, 22 (4), 313 (April 3, 1986).

Mono- and di-ketones have also previously been described for use as photoinitiators in addition-polymerizable compositions. References relating to such compositions include U.S. Pat. Nos. 3,427,161, 3,756,827, 3,759,807 and 4,071,424; U.K. Pat. Specification No. 1,304,112; European Published Pat. Appl. No. 150,952 and *Chem. Abs.* 95:225704U.

## SUMMARY OF THE INVENTION

The present invention provides, in one aspect, a coated abrasive having abrasive granules which are supported on and adherently bonded to at least one major surface of a backing sheet by a make coating of a first resinous material and a size coating of a second resinous material, said first and/or said second resinous materials being made by photocuring an addition-polymerizable composition comprising:

(a) free-radically-polymerizable monomer ("monomer"), and

(b) photoinitiator system, soluble in said monomer, comprising photochemically effective amounts of

(i) diaryliodonium salt ("iodonium salt"),

(ii) sensitizing compound ("sensitizer") capable of absorbing light somewhere within the range of wavelengths between about 300 and about 1000

nanometers and capable of sensitizing 2-methyl-4,6-bis(trichloromethyl)-s-triazine, and  
(iii) electron donor compound ("donor"), said donor being different from said sensitizing agent and wherein zero <math>E\_{ox}(\text{donor}) \leq E\_{ox}(\text{p-dimethoxybenzene})

The abrasive binders used in the invention have a very useful combination of cure speed, cure depth and shelf life. They cure well even when loaded with large amounts of mineral grain or with coarse grades of minerals.

The invention also provides a method for manufacturing coated abrasives.

DETAILED DESCRIPTION OF THE  
INVENTION

Aside from the abrasive binder (described in more detail below), the other components of the coated abrasive product of the invention can be selected from those typically used in the art. In that regard, see W. G. Pinkston, "Abrasives", *Kirk-Othmer Encyclopedia of Chemical Technology*, 3d Ed., 6, 26-52 (1978). The backing

can be formed of paper, resin-impregnated cloth, vulcanized fiber, film or any other backing material capable of supporting abrasive grains. The abrasive granules can be of any conventional grade utilized in the formation of coated abrasives and can be formed of flint, garnet, aluminum oxide, alumina:zirconia, synthetic ceramic, diamond, silicon carbide, etc., or mixtures thereof. The frequency of the abrasive granules on the sheet and their average particle size and size distribution can be conventional. The abrasive granules can be oriented or can be applied to the backing without orientation, depending upon the requirements of the particular coated abrasive product. Either the make coat or the size coat

of the coated abrasive product can be made using a conventional resinous material, the remaining coat

being made using a photochemically-initiated binder of

the invention. Both the make and size coat can be made using a binder of the invention.

The use of the binder of the present invention avoids many of the problems that plague binders generally used in coated abrasives. The binder does not require prolonged heating and/or dwell times before subsequent coatings are applied to the make coat. Unlike glue, the cured binder of the invention is unaffected by moisture. In fact, coated abrasive products made from the binder of the invention perform well under wet grinding conditions. Unlike varnish, the binder of the invention can be applied with little or no solvent and can be cured in a much shorter processing time. Varnish softens during wet grinding while the binder of the invention is not deleteriously affected. Curing of the binder of the invention is accomplished much more rapidly than curing of phenolic resin.

The coated abrasive product of the invention can also include such modifications as are known in the art. For example, a back coating such as pressure-sensitive adhesive can be applied to the nonabrasive side of the backing and various supersizes can be applied to the abrasive surface, such as zinc stearate to prevent abrasive loading, and others.

Turning now to the composition of the binder, a wide variety of monomers can be employed. Suitable monomers contain at least one ethylenically-unsaturated double bond, can be oligomers, and are capable of undergoing addition polymerization. Such monomers include mono-, di- or poly-acrylates and methacrylates such as methyl acrylate, methyl methacrylate, ethyl acrylate,

isopropyl methacrylate, n-hexyl acrylate, stearyl acrylate, allyl acrylate, glycerol diacrylate, glycerol triacrylate, ethyleneglycol diacrylate, diethyleneglycol diacrylate, triethyleneglycol dimethacrylate, 1,3-propanediol diacrylate, 1,3-propanediol dimethacrylate, trimethylolpropane triacrylate, 1,2,4-butanetriol trimethacrylate, 1,4-cyclohexanediol diacrylate, pentaerythritol triacrylate, pentaerythritol tetraacrylate, pentaerythritol tetramethacrylate, sorbitol hexacrylate, bis[1-(2-acryloxy)]-p-phenoxyphenyldimethylmethane, bis[1-(3-acryloxy-2-hydroxy)]-p-propoxyphenyldimethylmethane, tris(hydroxyethyl)-isocyanurate triacrylate; the bis-acrylates and bis-methacrylates of polyethylene glycols of molecular weight 200-500, copolymerizable mixtures of acrylated monomers such as those of U.S. Pat. No. 4,652,274, and acrylated oligomers such as those of U.S. Pat. No. 4,642,126; unsaturated amides such as methylene bis-acrylamide, methylene bis-methacrylamide, 1,6-hexamethylene bis-acrylamide, diethylene triamine tris-acrylamide and beta-methacrylaminoethyl methacrylate; and vinyl compounds such as styrene, diallyl phthalate, divinyl succinate, divinyl adipate and divinylphthalate. Mixtures of two or more monomers can be used if desired.

The monomer is combined with a three component or ternary photoinitiator system. The first component in the photoinitiator system is the iodonium salt, i.e., a diaryliodonium salt. The iodonium salt should be soluble in the monomer and preferably is shelf-stable (i.e., does not spontaneously promote polymerization) when dissolved therein in the presence of the sensitizer and donor. Accordingly, selection of a particular iodonium salt may depend to some extent upon the particular monomer, sensitizer and donor chosen. Suitable iodonium salts are described in U.S. Pat. Nos. 3,729,313, 3,741,769, 3,808,006, 4,250,053 and 4,394,403, the iodonium salt disclosures of which are incorporated herein by reference. The iodonium salt can be a simple salt (e.g., containing an anion such as  $\text{Cl}^-$ ,  $\text{Br}^-$ ,  $\text{I}^-$  or  $\text{C}_6\text{H}_5\text{SO}_3^-$ ) or a metal complex salt (e.g., containing an anion such as  $\text{BF}_4^-$ ,  $\text{PF}_6^-$ ,  $\text{SbF}_6^-$ ,  $\text{SbF}_5\text{OH}^-$  or  $\text{AsF}_6^-$ ). Mixtures of iodonium salts can be used if desired.

Preferred iodonium salts include diphenyliodonium salts such as diphenyliodonium chloride, diphenyliodonium hexafluorophosphate and diphenyliodonium tetrafluoroborate.

The second component in the photoinitiator system is the sensitizer. The sensitizer should be soluble in the monomer, and is capable of light absorption somewhere within the range of wavelengths between about 300 and about 1000 nanometers, more preferably about 400 and about 700 nanometers and most preferably about 400 to about 600 nanometers. The sensitizer is also capable of sensitizing 2-methyl-4,6-bis(trichloromethyl)-s-triazine, using the test procedure described in U.S. Pat. No. 3,729,313. Using currently available materials, that test is carried out as follows. A standard test solution is prepared having the following composition:

5.0 parts of a 5% (weight by volume) solution in methanol of 45,000-55,000 molecular weight, 9.0-13.0% hydroxyl content polyvinyl butyral ("Butvar B76", Monsanto)

0.3 parts trimethylolpropane trimethacrylate

0.03 parts 2-methyl-4,6-bis(trichloromethyl)-s-triazine (see *Bull. Chem. Soc. Japan*, 42, 2924-2930, 1969).

To this solution is added 0.01 parts of the compound to be tested as a sensitizer. The solution is knife-coated

onto a 0.05 mm clear polyester film using a knife orifice of 0.05 mm, and the coating is air dried for about 30 minutes. A 0.05mm clear polyester cover film is carefully placed over the dried but soft and tacky coating with minimum entrapment of air. The resulting sandwich construction is then exposed for three minutes to 161,000 Lux of incident light from a tungsten light source providing light in both the visible and ultraviolet range ("FCH" 650 watt quartz-iodine lamp, General Electric).

Exposure is made through a stencil so as to provide exposed and unexposed areas in the construction. After exposure the cover film is removed and the coating is treated with a finely divided colored powder, such as a color toner powder of the type conventionally used in xerography. If the tested compound is a sensitizer, the trimethylolpropane trimethacrylate monomer will be polymerized in the light-exposed areas by the light-generated free radicals from the 2-methyl-4,6-bis(trichloromethyl)-s-triazine. Since the polymerized areas will be essentially tack-free, the colored powder will selectively adhere only to the tacky, unexposed areas of the coating, providing a visual image corresponding to that in the stencil.

Preferably, in addition to passing the above test, a sensitizer is also selected based in part upon shelf stability considerations. Accordingly, selection of a particular sensitizer may depend to some extent upon the particular monomer, iodonium salt and donor chosen.

Suitable sensitizers are believed to include compounds in the following categories: ketones, coumarin dyes (e.g., ketocoumarins), xanthene dyes, acridine dyes, thiazole dyes, thiazine dyes, oxazine dyes, azine dyes, aminoketone dyes, porphyrins, aromatic polycyclic hydrocarbons, p-substituted aminostyryl ketone compounds, aminotriaryl methanes, merocyanines, squarylium dyes and pyridinium dyes. Ketones (e.g. monoketones or alpha-diketones) are preferred sensitizers. For applications requiring deep cure (e.g., cure of thick-section abrasives) it is preferred to employ sensitizers having an extinction coefficient below about 1000, more preferably below about 100, at the desired wavelength of irradiation for photopolymerization.

By way of example, a preferred class of ketone sensitizers has the formula:



where X is CO or  $\text{CR}^1\text{R}^2$ , where  $\text{R}^1$  and  $\text{R}^2$  can be the same or different, and can be hydrogen, alkyl, alkaryl or aralkyl, b is zero or 1, and A and B can be the same or different and can be substituted (having one or more non-interfering substituents) or unsubstituted aryl, alkyl, alkaryl, or aralkyl groups, or together A and B can form a cyclic structure which can be a substituted or unsubstituted cycloaliphatic, aromatic, heteroaromatic or fused aromatic ring.

Suitable ketones of the above formula include monoketones (b=0) such as 2,2-, 4,4- or 2,4-dihydroxybenzophenone, di-2-pyridyl ketone, di-2-furanyl ketone, di-2-thiophenyl ketone, benzoin, fluorenone, chalcone, Michler's ketone, 2-fluoro-9-fluorenone, 2-chlorothioxanthone, acetophenone, benzophenone, 1- or 2-acetonaphthone, 9-acetylanthracene, 2-, 3- or 9-acetylphenanthrene, 4-acetyl biphenyl, propiophenone, n-butyrophenone, valerophenone, 2-, 3- or 4-acetylpyridine, 3-acetyl coumarin and the like. Suitable diketones include aralkyldiketones such as anthraquinone, phen-

anthrenequinone, o-, m- and p-diacetylbenzene, 1,3-, 1,4-, 1,5-, 1,6-, 1,7- and 1,8-diacetyl naphthalene, 1,5-, 1,8- and 9,10-diacetylanthracene, and the like. Suitable  $\alpha$ -diketones ( $b=1$  and  $x=CO$ ) include 2,3-butanedione, 2,3-pantanedi one, 2,3-hexanedi one, 3,4-hexanedi one, 2,3-heptanedi one, 3,4-heptanedi one, 2,3-octanedi one, 4,5-octanedi one, benzil, 2,2'-, 3,3'- and 4,4'-dihydroxybenzil, furil, di-3,3'-indolylethanedione, 2,3-bornanedione (camphorquinone), biacetyl, 1,2-cyclohexanedi one, 1,2-naphthaquinone, acenaphthaquinone, and the like.

The third component in the photoinitiator system is the electron donor. A wide variety of donors can be employed. The donor is soluble in the monomer, and should meet the oxidation potential ( $E_{ox}$ ) limitation discussed in more detail below. Preferably, the donor also is selected based in part upon shelf stability considerations. Accordingly, selection of a particular donor may depend in part on the monomer, iodonium salt and sensitizer chosen. Suitable donors are capable of increasing the speed of cure or depth of cure of the binder of the invention upon exposure to light of the desired wavelength. Also, the donor has an  $E_{ox}$  greater than zero and less than or equal to  $E_{ox}$ (p-dimethoxybenzene). Preferably  $E_{ox}$  (donor) is between about 0.5 and 1 volts vs. a saturated calomel electrode ("S.C.E.").  $E_{ox}$  (donor) values can be measured experimentally, or obtained from references such as N. L. Weinburg, Ed., *Technique of Electroorganic Synthesis Part II Techniques of Chemistry*, Vol. V (1975), and C. K. Mann and K. K. Barnes, *Electrochemical Reactions in Nonaqueous Systems* (1970).

Preferred donors include amines (including aminoaldehydes and aminosilanes), amides (including phosphoramides), ethers (including thioethers), ureas (including thioureas), ferrocene, sulfonic acids and their salts, salts of ferrocyanide, ascorbic acid and its salts, dithiocarbamic acid and its salts, salts of xanthates, salts of ethylene diamine tetraacetic acid and salts of tetraphenylboronic acid. The donor can be unsubstituted or substituted with one or more non-interfering substituents. Particularly preferred donors contain an electron donor atom such as a nitrogen, oxygen, phosphorus, or sulfur atom, and an abstractable hydrogen atom bonded to a carbon or silicon atom alpha to the electron donor atom.

Preferred amine donor compounds include alkyl-, aryl-, alkaryl- and aralkyl-amines such as methylamine, ethylamine, propylamine, butylamine, triethanolamine, amylamine, hexylamine, 2,4-dimethylaniline, 2,3-dimethylaniline, o-, m- and p-toluidine, benzylamine, amino-pyridine, N,N'-dimethylethylenediamine, N,N'-diethylethylenediamine, N,N'-dibenzylethylenediamine, N,N'-diethyl-1,3-propanediamine, N,N'-diethyl-2-butene-1,4-diamine, N,N'-dimethyl-1,6-hexanediamine, 55 piperazine, 4,4'-trimethylenedipiperidine,

4,4-ethylenedipiperidine, p-N,N-dimethylamino-phenethanol and p-N,N-dimethylaminobenzonitrile; aminoaldehydes such as p-N,N-dimethylaminobenzaldehyde, p-N,N-diethylaminobenzaldehyde, 9-julolidine carboxaldehyde and 4-morpholinobenzaldehyde; and aminosilanes such as trimethylsilylmorpholine, trimethylsilylpiperidine, bis(dimethylamino)diphenylsilane, tris(dimethylamino)methylsilane, N,N-diethylaminotrimethylsilane, tris(dimethylamino)phenylsilane, tris(methylsilyl)amine, tris(dimethylsilyl)amine, bis(dimethylsilyl)amine, N,N-bis(dimethylsilyl)aniline, N-phenyl-N-dimethylsilylaniline and N,N-dimethyl-N-

dimethylsilylamine. Tertiary aromatic alkylamines, particularly those having at least one electron-withdrawing group on the aromatic ring, have been found to provide especially good shelf stability. Good shelf stability has also been obtained using amines that are solids at room temperature.

Preferred amide donor compounds include N,N-dimethylacetamide, N,N-diethylacetamide, N-methyl-N-phenylacetamide, hexamethylphosphoramide, hexaethylphosphoramide, hexapropylphosphoramide, trimorpholinophosphine oxide and triperidinophosphine oxide.

Suitable ether donor compounds include 4,4'-dimethoxybiphenyl, 1,2,4-trimethoxybenzene and 1,2,4,5-tetramethoxybenzene.

Suitable urea donor compounds include N,N'-dimethylurea, N,N-dimethylurea, N,N'-diphenylurea, tetramethylthiourea, tetraethylthiourea, tetra-n-butylthiourea, N,N-di-n-butylthiourea, N,N'-di-n-butylthiourea, N,N-diphenylthiourea and N,N'-diphenyl-N,N'-diethylthiourea.

The three components of the photoinitiator system are present in "photochemically effective amounts", that is, amounts of each component sufficient to enable the binder to undergo photochemical hardening upon exposure to light of the desired wavelength. Preferably, for every 100 parts of monomer, the binder of the invention contains about 0.005 to about 10 parts (more preferably about 0.1 to about 4 parts) each of iodonium salt, sensitizer and donor. The amounts of each component are independently variable and thus need not be equal, with larger amounts generally providing faster cure, but shorter shelf life. Sensitizers with high extinction coefficients (e.g., above about 10,000) at the desired wavelength of irradiation for photopolymerization generally are used in reduced amounts.

The binders of the invention can contain a wide variety of adjuvants depending upon the desired end use. Suitable adjuvants include solvents, diluents, resins, thermally-cured binders, plasticizers, pigments, dyes, inorganic or organic reinforcing or extending fillers (at preferred amounts of about 10% to about 90% by weight, based on the total weight of the composition), thixotropic agents, indicators, inhibitors, stabilizers, UV absorbers, and the like. The amounts and types of such adjuvants, and their manner of addition to a composition of the invention will be familiar to those skilled in the art.

The binders of the invention can be cured using a variety of methods. It is convenient to employ light sources that emit ultraviolet or visible light such as quartz halogen lamps, tungsten-halogen lamps, mercury arcs, carbon arcs, low-, medium-, and high-pressure mercury lamps, plasma arcs, light emitting diodes and lasers. Electron beam ("E-beam") irradiation and other curing devices that do not depend on light emission can also be employed. In general, heat or an inert atmosphere will accelerate cure.

The following examples are offered to aid in understanding the invention and are not to be construed as limiting the scope thereof. Unless otherwise indicated, all parts and percentages are by weight.

#### EXAMPLE 1

Three stock solutions were prepared from 0.25 parts camphorquinone (CPQ), 50 parts triethyleneglycol dimethacrylate (TEGDMA) and 50 parts bisphenol A diglycidyl ether dimethacrylate (BisGMA). 0.50 Part

diphenyliodonium hexafluorophosphate ( $\phi_2\text{I}^+\text{PF}_6^-$ ) was added to the first solution. 0.25 Part sodium p-toluenesulfinate (STS) was added to the second solution. 0.50 Part  $\phi_2\text{I}^+\text{PF}_6^-$  and 0.25 part STS were added to the third solution. Each solution was poured into a 6 mm diameter "Teflon" mold to a depth of 2.5 mm, covered with polyester film and irradiated for 10 seconds using a handheld visible light curing lamp ("Visilux", 3M) whose lightguide output end was placed directly on the polyester film.

The solutions containing only CPQ and  $\phi_2\text{I}^+\text{PF}_6^-$  or CPQ and STS formed a soft gel. The solution containing CPS,  $\phi_2\text{I}^+\text{PF}_6^-$  and STS hardened to a solid having a Barcol hardness of 40 (ASTM D-2583) on both its top and bottom surfaces.

In a further experiment, three stock solutions were prepared from 11.85 parts each of the above monomers,

## EXAMPLE 2

Equimolar amounts of a variety of donors were added to monomer stock solutions containing 50 parts trimethylolpropane trimethacrylate, 50 parts 1,4-butanediol dimethacrylate, 0.25 part CPQ and optionally 0.5 part of the iodonium salt  $\phi_2\text{I}^+\text{PF}_6^-$ .

The resulting solutions were irradiated with visible light at an intensity of 60 mW/cm<sup>2</sup> (as measured by a United Detector Technology Model 351 portable photometer/radiometer) at 400-500 nm. The solutions were stirred using a glass rod and the time required to reach the gelation point was recorded. Set out below in TABLE I are the run number, donor compound,  $E_{ox}$  (donor), weight percent donor, and gel times for solutions prepared with and without the iodonium salt. The donors are listed in TABLE I in order of generally decreasing oxidation potential.

TABLE I

| Run No. | Donor                            | $E_{ox}$ (donor) | % donor | Gel time, seconds |                                |
|---------|----------------------------------|------------------|---------|-------------------|--------------------------------|
|         |                                  |                  |         | Sensitizer/donor  | Sensitizer/donor/iodonium salt |
| 1       | control                          |                  | 0       | >200              | 190                            |
| 2       | acetonitrile                     | 2.60             | 0.124   | >200              | >190                           |
| 3       | nitrobenzene                     |                  | 0.373   | >200              | >190                           |
| 4       | methylethylketone                |                  | 0.218   | >200              | >190                           |
| 5       | 2,5-dimethyl-2,4-hexadiene       | 2.10             | 0.334   | >200              | >190                           |
| 6       | ethylmethylthioacetate           | 1.70             | 0.407   | >200              | >190                           |
| 7       | p-bromothioanisole               | 1.60             | 0.615   | >200              | >190                           |
| 8       | 3,3'-dimethoxybiphenyl           | 1.60             | 0.649   | >200              | >190                           |
| 9       | tetrahydrofuran                  | 1.60             | 0.220   | >200              | >190                           |
| 10      | hexaethylbenzene                 | 1.49             | 0.492   | >200              | >190                           |
| 11      | methoxyphenylphenylether         |                  | 0.604   | >200              | 188                            |
| 12      | p-dimethoxybenzene               | 1.34             | 0.418   | 205               | 160                            |
| 13      | N,N-dimethylacetamide            | 1.32             | 0.264   | 204               | 150                            |
| 14      | phenylacetate                    | 1.30             | 0.413   | >200              | >190                           |
| 15      | n-propylamine                    | 1.30             | 0.200   | 90                | 24                             |
| 16      | aniline                          | 1.28             | 0.282   | >200              | >190                           |
| 17      | 1,3-dibutylthiourea              |                  | 0.570   | >200              | 137                            |
| 18      | tetramethylurea                  |                  | 0.352   | 94                | 101                            |
| 19      | tetrabutylthiourea               |                  | 0.909   | 38                | 29                             |
| 20      | dipentylamine                    | 1.22             | 0.477   | 159               | 19                             |
| 21      | 1,2,4-trimethoxybenzene          | 1.12             | 0.509   | >225              | 55                             |
| 22      | hexamethylphosphoramide          | 1.00             | 0.543   | 80                | 50                             |
| 23      | tripiperidinophosphine oxide     | 1.00             | 0.907   | 52                | 40                             |
| 24      | trimethylsilyl morpholine        |                  | 0.483   | 112               | 21                             |
| 25      | N,N-dimethylbenzylamine          | 1.00             | 0.410   | 18                | 8                              |
| 26      | tris-dimethylsilylamine          |                  | 0.580   | 108               | 32                             |
| 27      | triethanolamine                  | 0.96             | 0.452   | 17                | 6                              |
| 28      | tris(dimethylamino)-phenylsilane |                  | 0.719   | 15                | 9                              |
| 29      | triphenylamine                   | 0.86             | 0.737   | >200              | >190                           |
| 30      | triphenylphosphine               |                  | 0.794   | >200              | 172                            |
| 31      | p-dimethylaminobenzaldehyde      | 0.70             | 0.452   | 13                | 11                             |
| 32      | N,N-dimethyl-p-toluidine         | 0.65             | 0.410   | 14                | 7                              |
| 33      | p-dimethylaminophenyl-alcohol    |                  | 0.65    | 0.500             | 13                             |

76 parts filler, and 0.25 part CPQ. 0.25 Part  $\phi_2\text{I}^+\text{PF}_6^-$  was added to the first solution. 0.25 Part N,N-dimethylaminophenethyl alcohol ("D-1") was added to the second solution. 0.25 Part  $\phi_2\text{I}^+\text{PF}_6^-$  and 0.25 part D-1 were added to the third solution. Each solution was cured in a mold as described above, but using a 6 mm deep mold and a 20 second cure time. The solution containing only  $\phi_2\text{I}^+\text{PF}_6^-$  did not cure. The solution containing only D-1 had top and bottom Barcol hardness values of 56 and 2, respectively. The solution containing both  $\phi_2\text{I}^+\text{PF}_6^-$  and D-1 had top and bottom Barcol hardness values of 60 and 30, respectively.

The above data illustrates that an increased degree of polymerization and depth of cure can be obtained using a binder of the invention.

The above data illustrates that an increased cure rate is obtained using a binder of the invention, and demonstrates the advantage of using donors whose  $E_{ox}$  value is less than or equal to that of p-dimethoxybenzene and that have an abstractable hydrogen atom on a carbon or silicon atom alpha to the donor atom.

## EXAMPLE 3

An unfilled binder formulation was prepared from the following ingredients:

|                                                  | % Solids |
|--------------------------------------------------|----------|
| acrylamide                                       | 43.3     |
| N,N'-methylenebisacrylamide                      | 4.3      |
| polyvinyl alcohol<br>(m.w. 2000, 75% hydrolyzed) | 51.9     |

in the visible region or 60 sec. in the ultraviolet region except as noted.

TABLE II

| Run<br>No. | Sensitizer                                                | Visible Light Sensitivity Enhancement |                      |                              | Sensitizer/<br>donor/<br>iodonium salt |
|------------|-----------------------------------------------------------|---------------------------------------|----------------------|------------------------------|----------------------------------------|
|            |                                                           | Sensitizer<br>$\lambda_{max}$ , nm    | Sensitizer/<br>donor | Sensitizer/<br>iodonium salt |                                        |
| 1          | methylene blue                                            | 661                                   | (c)                  | 3                            | 12                                     |
| 2          | toluidine blue                                            | 626                                   | 6                    | (c)                          | 16                                     |
| 3          | rose bengal                                               | 548                                   | (d)                  | (c)                          | 16                                     |
| 4          | phenosafranine                                            | 520                                   | (d)                  | (c)                          | 9                                      |
| 5          | 1,3-bis(4-dimethylaminobenzylidene)acetone <sup>(a)</sup> | 434                                   | (d)                  | 11                           | 17                                     |
| 6          | tris(bipyridyl)ruthenium (+2) chloride                    | 453                                   | (d)                  | (c)                          | 12                                     |
| 7          | crystal violet <sup>(b)</sup>                             | 593                                   | (d)                  | (c)                          | 10                                     |
| 8          | eosin yellow                                              | 517                                   | (c)                  | 4                            | 12                                     |
| 9          | 3,3'-dimethylthiocarbocyanine iodide <sup>(a)</sup>       | 553                                   | (d)                  | (c)                          | 12                                     |

Notes to TABLE II:

<sup>(a)</sup>5 sec. exposure.<sup>(b)</sup>60 sec. exposure.<sup>(c)</sup>Image lost during development.<sup>(d)</sup>No image formed.

TABLE III

| Run<br>No. | Sensitizer                                          | Ultraviolet Light Sensitivity Enhancement |                      |                              | Sensitizer/<br>donor/<br>iodonium salt |
|------------|-----------------------------------------------------|-------------------------------------------|----------------------|------------------------------|----------------------------------------|
|            |                                                     | Sensitizer<br>$\lambda_{max}$ , nm        | Sensitizer/<br>donor | Sensitizer/<br>iodonium salt |                                        |
| 1          | 2,5-bis(cinamylidene)cyclopentanone                 | 400                                       | (b)                  | (b)                          | 8                                      |
| 2          | 4'-methoxybenzylidene-4-nitro-acetophenone          | 356                                       | (b)                  | (b)                          | 11                                     |
| 3          | 2-(4-dimethylaminobenzylidene)-<br>dimethylmalonate | 377                                       | (b)                  | (c)                          | 5                                      |
| 4          | Michler's ketone <sup>(a)</sup>                     | 355                                       | (b)                  | 10                           | 15                                     |
| 5          | 2-chlorothioxanthone                                | 387                                       | (b)                  | (c)                          | 11                                     |

Notes to TABLE III:

<sup>(a)</sup>15 Second exposure at 40% power.<sup>(b)</sup>No image formed.<sup>(c)</sup>Image lost during development.

| % Solids                    |     |
|-----------------------------|-----|
| surfactant ("Triton X-100") | 0.5 |

made up to 11.5% solids in a 1/1 v/v acetonitrile/water mixture. Using a red safelight, coating samples were prepared by combining 25 ml portions of the above stock solution with 0.01 g of the sensitizer and optionally adding 0.1 g  $\phi_2I^+PF_6^-$  and/or 0.1 g STS. The samples were coated onto gelatin-subbed polyester film using a #18 wire wound rod, dried with a heat gun, then oven-dried for 2 minutes at 60° C. The coated films were exposed under vacuum through a 21 step sensitivity guide, using a tungsten ("Model 70" Transparency Maker, 3M) or ultraviolet (2Kw Berkey Ascor, Berkey Technical Company) light source. The exposed samples were developed using a 3/20, v/v water/methanol solvent mixture. Relative speed was determined by the number of steps (average of 3 samples) remaining after development. Set out below in TABLE II are the results for the samples exposed to visible light, and set out below in TABLE III are the results for the samples exposed to ultraviolet light. Each exposure was 30 sec.

The above data illustrates that combination of an iodonium salt, sensitizer and donor can increase cure speed by one to two orders of magnitude compared to compositions containing only sensitizer and donor or only sensitizer and iodonium salt.

## EXAMPLE 4

To illustrate the effect of  $E_{ox}$  (donor) upon cure speed, a series of compositions was evaluated as follows. A monomer stock solution was prepared from 10% pentaerythritol tetraacrylate in 4/1, w/w, acetonitrile/water. To 3 ml portions of this solution in 13×100 mm "Pyrex" test tubes were added about 0.02 g of  $\phi_2I^+PF_6^-$  and/or a donor compound and enough sensitizer to give an optical density of between 1 and 2, as evaluated visually. The solutions were purged with  $N_2$  for 2 minutes before and continuously during light irradiation. The light source was a Kodak "Carousel" Projector lamp equipped with a 440 nm filter. Relative speed was determined by measuring gelation time.

Set out below in TABLE IV are the run number, the sensitizers and their  $\lambda_{max}$  values, the donor compounds and their  $E_{ox}$  values, and the gelation times for solutions containing iodonium salt plus sensitizer, sensitizer plus donor, or iodonium salt plus sensitizer plus donor.

TABLE IV

| Run<br>No. | Sensitizer     | Gel time, sec.  |                      |                                 |                           |                                        |
|------------|----------------|-----------------|----------------------|---------------------------------|---------------------------|----------------------------------------|
|            |                | $\lambda_{max}$ | Donor <sup>(a)</sup> | Iodonium<br>salt/<br>sensitizer | Sensi-<br>tizer/<br>Donor | Iodonium salt/<br>sensitizer/<br>donor |
| 1          | methylene blue | 661             | STS                  | (b)                             | (b)                       | 10                                     |

TABLE IV-continued

| Run No. | Identity                                                      | Sensitizer | $\lambda_{max}$ | Donor <sup>(a)</sup> | Gel time, sec.               |                           |                                        |
|---------|---------------------------------------------------------------|------------|-----------------|----------------------|------------------------------|---------------------------|----------------------------------------|
|         |                                                               |            |                 |                      | Iodonium salt/<br>sensitizer | Sensi-<br>tizer/<br>Donor | Iodonium salt/<br>sensitizer/<br>donor |
| 2       | thionin                                                       |            | 598             | STS                  | (b)                          | (b)                       | 180                                    |
| 3       | thionin                                                       |            | 598             | FC                   | (c)                          | (c)                       | <5                                     |
| 4       | phenosafranine                                                |            | 520             | STS                  | (b)                          | (b)                       | 15                                     |
| 5       | rose bengal                                                   |            | 548             | STS                  | (b)                          | 30                        | <5                                     |
| 6       | fluorescein                                                   |            | 491             | STS                  | (b)                          | (b)                       | 15                                     |
| 7       | crystal violet                                                |            | 588             | STS                  | (b)                          | (b)                       | >300                                   |
| 8       | crystal violet                                                |            | 588             | FC                   | (c)                          | (c)                       | 120                                    |
| 9       | malachite green                                               |            | 614             | STS                  | (b)                          | (b)                       | >300                                   |
| 10      | malachite green                                               |            | 614             | FC                   | (c)                          | (c)                       | 60                                     |
| 11      | 3,3'-dimethylthiocarbocyanine iodide                          |            | 553             | STS                  | 60                           | (b)                       | 30                                     |
| 12      | 2,6-bis(4-dimethylaminostyryl)-1-methyl-<br>pyridinium iodide |            | 490             | STS                  | (b)                          | (b)                       | (b)                                    |
| 13      | 2,6-bis(4-dimethylaminostyryl)-1-methyl-<br>pyridinium iodide |            | 490             | FC                   | (c)                          | (c)                       | 90                                     |
| 14      | tris(bipyridyl)ruthenium (+2) chloride                        |            | 453             | STS                  | 60                           | 60                        | <10                                    |
| 15      | 1-methyldiaminoanthraquinone                                  |            | 502             | STS                  | (b)                          | (b)                       | 45                                     |
| 16      | 1,2,2-tricyano-1-(4-dimethylaminophenyl)ethylene              |            | 525             | STS                  | (b)                          | (b)                       | (b)                                    |
| 17      | 1,2,2-tricyano-1-(4-dimethylaminophenyl)ethylene              |            | 525             | FC                   | (c)                          | (c)                       | 90                                     |

## Notes to TABLE IV:

<sup>(a)</sup>STS = sodium p-toluenesulfinate ( $E_{ox}$  = 0.76); FC = ferrocyanide ( $E_{ox}$  = 0.2).<sup>(b)</sup>No reaction.<sup>(c)</sup>Not determined.

The above data illustrates that when  $E_{ox}$  (donor) is decreased, cure speed generally increases (see also TABLE I).

## EXAMPLE 5

A polyester cloth backing (woven, spun polyester cloth, 0.03 g/cm<sup>2</sup>, Milliken) was impregnated with resin by saturating the backing with an ultraviolet-light-curable resin mixture made by combining 75 parts epoxy-acrylate resin ("Novacure 3500", Interez), 15 parts pentaerythritol triacrylate, 9 parts n-vinyl pyrrolidone and 1 part  $\alpha$ ,  $\alpha$ -dimethoxy- $\alpha$ -phenyl acetophenone, and curing the resin under ultraviolet light in air using an energy density of 0.3 J/cm<sup>2</sup>.

A coated abrasive binder resin was prepared from a 50:50 mixture of the triacrylate of tris-hydroxyethylisocyanurate and the triacrylate of trimethylolpropane, filled to 50% with calcium carbonate. 0.25 Part each of  $\phi_2I^+PF_6^-$ , CPQ and D-1 were mixed into the binder resin.

The resin-impregnated backing was knife-coated with the binder resin at a coating thickness of 0.1 mm, then drop-coated with grade 50 Al<sub>2</sub>O<sub>3</sub> mineral. The binder was cured under nitrogen in 5 to 10 seconds using a high intensity visible light source (Model F440 with 4V678 lamp, Fusion Systems) operated at a distance of about 15 cm. Microscopic examination of the cured abrasive showed that cure took place throughout the binder, even underneath individual mineral granules. By comparison, if the photoinitiator system was excluded from the resin and a 5Mrad dose of E-beam irradiation (250 Kv acceleration potential) was employed to effect cure, pools of wet uncured resin remained under individual mineral granules and the granules were poorly adhered on the backing.

A sample of the coated abrasive was size coated with the same resin system, using a coating weight just sufficient to coat the mineral granules. The size coat was cured under the visible light source used to cur the make coat. The resulting coated abrasive was evaluated using a reciprocating grinding apparatus ("rocker 65 drum") on a 6 mm thick 1018 carbon steel workpiece. After 500 cycles, no shelling was observed and an average of 0.77 g of steel was removed. A comparison abra-

sive sample was prepared using a make coat that contained the same photoinitiator system (cured using visible light), and a size coat that did not contain the photoinitiator system (cured using E-beam). The comparison abrasive shelled after only 20 cycles and removed only 0.02 g of steel.

Comparable results were obtained when sensitizers such as benzil, 2-chlorothioxanthone and fluorenone were substituted for camphorquinone. Improved uncured resin shelf life and ambient light stability were obtained when donor compounds such as ethyl p-dimethylaminobenzoate, p-dimethylaminobenzaldehyde and p-dimethylaminobenzonitrile were substituted for p-dimethylaminophenethyl alcohol.

The above-described abrasive binder system should be a useful substitute for standard phenolic-based binders, and could offer reduced energy consumption and higher throughput during manufacture.

Various modifications and alterations of this invention will be apparent to those skilled in the art without departing from the scope and spirit of this invention. It should be understood that this invention is not limited to the illustrative embodiments set forth herein.

## We claim:

1. A coated abrasive having abrasive granules which are supported on and adherently bonded to at least one major surface of a backing sheet- by a make coating of a first resinous material and a size coating of a second resinous material, said first and/or said second resinous materials being made by photocuring an addition-polymerizable composition comprising:

- (a) free-radically-polymerizable monomer, and
- (b) photoinitiator system, soluble in said monomer, comprising photochemically effective amounts of
  - (i) aryliodonium salt,
  - (ii) sensitizing compound capable of absorbing light somewhere within the range of wavelengths between about 300 and about 1000 nanometers and capable of sensitizing 2-methyl-4,6-bis(trichloromethyl)-s-triazine, and
  - (iii) electron donor compound, said donor being different from said sensitizing compound and zero  $<E_{ox}$  (donor)  $\leq E_{ox}$  (p-dimethoxybenzene).

2. A coated abrasive according to claim 1, wherein said abrasive granules are selected from the group consisting of flint, garnet, aluminum oxide, alumina:zirconia, synthetic ceramic, diamond and silicon carbide.

3. A coated abrasive according to claim 1, wherein said backing sheet comprises paper, resin-impregnated cloth, vulcanized fiber or film.

4. A coated abrasive according to claim 1, wherein said first resinous binder comprises said addition-polymerizable composition, and said second resinous binder is selected from the group consisting of said addition-polymerizable composition, varnish, epoxy resin, phenolic resin and polyurethane.

5. A coated abrasive according to claim 1, wherein said first resinous binder is selected from the group consisting of said addition-polymerizable composition, glue, varnish, epoxy resin, phenolic resin and polyurethane, and said second resinous material comprises said addition-polymerizable composition.

6. A coated abrasive according to claim 1, wherein said monomer comprises an acrylated oligomer.

7. A coated abrasive according to claim 1, wherein said monomer comprises the triacrylate of tris-hydroxyethylisocyanurate and/or the triacrylate of trimethylolpropane.

8. A coated abrasive according to claim 1, wherein said aryliodonium salt comprises a diphenyliodonium simple salt or diphenyliodonium metal complex salt.

9. A coated abrasive according to claim 1, wherein said range of wavelengths is about 400 to about 700 nanometers.

10. A coated abrasive according to claim 1, wherein said range of wavelengths is about 400 to about 600 nanometers.

11. A coated abrasive according to claim 1, wherein said sensitizing compound comprises a ketone.

12. A coated abrasive according to claim 11, wherein said sensitizing compound comprises an  $\alpha$ -diketone having an extinction coefficient below about 1000 at the wavelength at which said addition-polymerizable composition is irradiated when photopolymerized.

13. A coated abrasive according to claim 11, wherein said sensitizing compound is selected from the group consisting of camphorquinone, benzil, 2-chlorothioxanthone and fluorenone.

14. A coated abrasive according to claim 11, wherein said sensitizing compound has the formula:



where X is CO or CR<sup>1</sup>R<sup>2</sup>, where R<sup>1</sup> and R<sup>2</sup> can be the same or different, and can be hydrogen, alkyl, alkaryl or aralkyl, b is zero or 1, and A and B can be the same or different and can be substituted or unsubstituted aryl, alkyl, alkaryl or aralkyl groups, or together A and B can form a cyclic structure which can be a substituted or unsubstituted cycloaliphatic, aromatic, heteroaromatic or fused aromatic ring.

15. A coated abrasive according to claim 1, wherein said E<sub>ox</sub>(donor) is between about 0.5 and 1 volts vs. a saturated calomel electrode.

16. A coated abrasive according to claim 1, wherein said donor is selected from the group consisting of amines, amides, ethers, ureas, ferrocene, sulfonic acids and their salts, salts of ferrocyanide, ascorbic acid and its salts, dithioca-rbamic acid and its salts, salts of xanthates, salts of ethylene diamine tetraacetic acid and salts of tetraphenylboronic acid.

17. A coated abrasive according to claim 1, wherein said donor contains a nitrogen, oxygen, phosphorus or sulfur donor atom and an abstractable hydrogen atom bonded to a carbon or silicon atom alpha to said donor atom.

18. A coated abrasive according to claim 1, wherein said donor comprises a tertiary amine containing an aromatic ring.

19. A coated abrasive according to claim 8, wherein there is at least one electron-withdrawing group on said aromatic ring.

20. A coated abrasive according to claim 1, wherein said composition contains, for every 100 parts by weight of said monomer, about 0.005 to about 10 parts, by weight each of said aryliodonium salt, said sensitizing compound and said donor.

21. A coated abrasive according to claim 20, wherein said composition contains, for every 100 parts by weight of said monomer, about 0.1 to about 4 parts by weight each of said aryliodonium salt, said sensitizing compound and said donor.

22. A coated abrasive having abrasive granules which are supported on and adherently bonded to at least one major surface of a backing sheet by a make coating of a first resinous material and a size coating of a second resinous material, said first and/or said second resinous materials being made by photocuring an addition-polymerizable composition comprising:

- (a) free-radically-polymerizable monomer, and
- (b) photoinitiator system, soluble in said monomer, comprising 0.1 to 4 parts each of
  - (i) diphenyliodonium metal complex salt,
  - (ii) ketone sensitizing compound capable of absorbing light somewhere within the range of wavelengths between about 400 and about 600 nanometers and capable of sensitizing 2-methyl-4,6-bis(trichloromethyl)-s-triazine, and
  - (iii) electron donor compound containing a nitrogen donor atom and having an abstractable hydrogen atom bonded to a carbon or silicon atom alpha to said nitrogen atom,

wherein said donor compound is different from said sensitizing compound and wherein about  $0.5 < E_{ox}(\text{donor}) \leq$  about 1 volt vs. a saturated calomel electrode.

23. A method for making coated abrasive products comprising the steps of

- (1) uniformly coating a backing sheet with a make coat of a first resinous material in liquid form;
- (2) depositing a plurality of abrasive granules uniformly over the surface of said make coat of first resinous material;
- (3) curing said first resinous material to adherently bond said granules to said backing sheet surface;
- (4) coating over said make coat and said granules with a size coat of a second resinous material; and
- (5) curing the resultant coated product until said second resinous material is solid,

wherein at least one of said first or second resinous binder materials is cured by irradiation with ultraviolet or visible light and comprises an addition-polymerizable composition comprising:

- (a) free-radically-polymerizable monomer, and
- (b) photoinitiator system, soluble in said monomer, comprising photochemically effective amounts
  - (i) aryliodonium salt
  - (ii) sensitizing compound capable of absorbing light somewhere within the range of wavelengths between about 300 and about 1000 nanometers

and capable of sensitizing 2-methyl-4,6-bis(trichloromethyl)-s-triazine, and  
(iii) electron donor compound, said donor being  
different from said sensitizing compound and  
zero  $\triangle E_{ox}$  (donor)  $\leq E_{ox}$  (p-dimethoxybenzene).  
24. A method according to claim 23, wherein said

sensitizing compound comprises a ketone having an  
extinction coefficient below about 1000 at the wave-  
length of said light.

\* \* \* \* \*

10

15

20

25

30

35

40

45

50

55

60

65

UNITED STATES PATENT AND TRADEMARK OFFICE  
CERTIFICATE OF CORRECTION

PATENT NO. : 4,735,632

DATED : April 5, 1988

INVENTOR(S) : Joel D. Oxman, F. Andrew UBel, III and Eric G. Larson

It is certified that error appears in the above-identified patent and that said Letters Patent is hereby corrected as shown below:

Column 4, lines 66-67, "2-, 3- or 4-acetylpyridine," should read -- 2-, 3- or 4-acetylpyridine, --.

Column 5, line 14, "employed" should be followed by a period.

Column 6, line 3, "t" should read --to--.

Column 10, line 58, " $\lambda_{\text{mas}}$ " should read -- $\lambda_{\text{max}}$ --.

Column 11, line 63, "cur" should read --cure--.

Column 12, line 52, "sheet-" should read --sheet--.

Column 13, line 53, "can-be" should read --can be--.

Column 13, line 66, "dithioca-rbamic" should read --dithiocarbamic--.

Signed and Sealed this  
Fourteenth Day of May, 1991

Attest:

HARRY F. MANBECK, JR.

Attesting Officer

Commissioner of Patents and Trademarks